

No. 822,212.

PATENTED MAY 29, 1906.

J. H. LUBBERS.

METHOD OF DRAWING SHEET GLASS.

APPLICATION FILED JAN. 12, 1903.

4 SHEETS—SHEET 1.

Fig. 1.



WITNESSES  
*J. H. Lubbers*  
Warren L. Swartz

INVENTOR  
*J. H. Lubbers*  
by DeKure & Reynolds  
his atty

No. 822,212.

PATENTED MAY 29, 1906

J. H. LUBBERS.

METHOD OF DRAWING SHEET GLASS.

APPLICATION FILED JAN. 12, 1903.

4 SHEETS—SHEET 2.



*L. A. Comer*  
Warren W. Gravity.

Fig. 2.

*J. H. Lubbers*  
by *Beckers & Synes*  
*his atto*

No. 822,212.

PATENTED MAY 29, 1906.

J. H. LUBBERS.

METHOD OF DRAWING SHEET GLASS.

APPLICATION FILED JAN. 12, 1903.

4 SHEETS—SHEET 3.



No. 822,212.

PATENTED MAY 29, 1906.

J. H. LUBBERS.

## METHOD OF DRAWING SHEET GLASS.

APPLICATION FILED JAN. 12, 1903.

4 SHEETS-SHEET 4.



**WITNESSES**

L. A. Rosner  
Warren W. Schwartz

Fig. 4.

**INVENTOR**

J. T. Lubbers  
by R. L. Nease & Hayes  
his attorney

# UNITED STATES PATENT OFFICE.

JOHN H. LUBBERS, OF ALLEGHENY, PENNSYLVANIA, ASSIGNOR TO  
JAMES A. CHAMBERS, TRUSTEE, OF PITTSBURG, PENNSYLVANIA.

## METHOD OF DRAWING SHEET-GLASS.

No. 822,212.

Specification of Letters Patent.

Patented May 29, 1906.

Application filed January 12, 1903. Serial No. 138,650.

*To all whom it may concern:*

Be it known that I, JOHN H. LUBBERS, of Allegheny, in the county of Allegheny and State of Pennsylvania, have invented a new and useful Method of Drawing Sheet-Glass, of which the following is a full, clear, and exact description, reference being had to the accompanying drawings, forming part of this specification, in which—

10 Figure 1 is a vertical cross-section through a furnace and drawing-chamber constructed in accordance with my invention. Fig. 2 is a longitudinal vertical section through the leer and drawing-chamber. Fig. 3 is a sectional plan view of the apparatus. Fig. 4 is a sectional side elevation. Fig. 5 is a detail view showing the lifting mechanism for the pot or trough, and Fig. 6 is a detail of a double cooling-pipe I employ.

20 My invention relates to the drawing of glass articles, such as sheets, and is designed to provide an improved method therefor.

25 The invention relates to an improved manner of filling and discharging the drawing pot or trough, to an improved manner of drawing a plurality of sheets simultaneously to avoid warping, and to the manner of annealing the glass.

In the drawings, 2 represents a forehearth 30 or extension of a tank 3, in which the glass rests at about the level indicated in Fig. 4. In this forehearth is provided a dipping-ladle 4, which normally rests in the position shown in Fig. 4, in which a slot 5 in the ladle allows 35 the glass to enter it, while its discharge-nozzle 6 rests upon another tilting trough 7. The ladle 4 is provided with a lower depending rib or projection 8, which when the ladle is lifted causes the glass on the lower side of the 40 ladle to drip back into the bath. I thus prevent the glass from entering the hinge or pivotal joint to freeze therein and prevent proper movement. The trough 7 has a depending portion 9, which hooks over the inner end of the outlet or tap-hole 10, which is 45 downwardly inclined to hold the trough 7 in inclined position when the receiving-pot 11 is lowered. The ladle is tilted by means of bars which are inserted through holes in the 50 side walls 12, which holes are normally closed by plugs or refractory slides 13. The bars enter pockets 14, molded in the sides of the ladle, and two operators may thus swing the ladle up, causing it to discharge its contents

into the trough 7 and thence into the pot 11, 55 which at this time is in the lowered horizontal position indicated by dotted lines.

The pot 11 is of general rectangular pan shape, is made of refractory material, and is preferably mounted upon vertically-movable 60 refractory posts 15 and 16, the post 15 being mounted on a transverse support 17, carried by the piston-rods of motive cylinders 18. The posts 16 are similarly supported, and their upper ends engage a rib or hinge portion 19 on the lower side of the pot. All of these supporting-posts project through the bottom 20 of a furnace-chamber, and by actuating one or both of the sets of cylinders 65 the pot may be moved vertically in parallel 70 lines or tilted to discharge its contents into a small receptacle 21 after the drawing operation.

The drawing-frame 22 is provided with corner-guides 23, which engage guide-posts 75 24 at the corners of the leer-chamber or drawing-chamber 25, which extends upwardly above the pot-chamber, and the end bars of the drawing-frame are provided with a series of vertical slots in which seat the parallel bars 26, carrying the tongs 27, between 80 which the bait of glass or other material 28 is secured. The frame may be raised and lowered by suitable means, such as flexible connections 29, extending up over pulleys 85 above the leer-chamber.

At the sides of the pot-chamber are provided swinging or sliding shields 30, of refractory material, secured to square water-cooled boxes or tubes 31, having rounded portions 90 32 extending through the side walls and connected with a water inlet and outlet. The end tube portions may be turned by the operator to swing the shield down and cover the pot or to swing them back into the position 95 shown, where they rest during drawing, cutting off the heat from the forehearth, the pot at this time being raised against the top plate 33.

To chill the sheets at or near the drawing-point, I provide a series of double water-cooled pipes 34, which extend between the baits and along the outside of the outer baits. Each water-pipe is supplied with water through a flexible connection 35 at one end with a header 36, water passing out at the 100 other end into another similar header 37, and a pipe of larger diameter surrounds the water-pipe and chills the sheets. This pre-

vents dripping of water from sweating, and the outer pipes are preferably of brass or non-corrosive material and may have centering devices to hold the inner pipes central. This 5 also prevents chilling of glass when the pipes are brought together.

In Fig. 2 I show the upper part of the drawing-chamber, with a part of the leer. In this figure, 38 is the first compartment of the leer, 10 which is separated from the drawing-chamber by a sliding door 39, movable sidewise on rollers 40, and this compartment is separated from the next compartment by a similar door 41. The leer is made up of a series of these 15 compartments, connecting with each other above the partitions and below the roof 42, and the compartments are heated by separate gas-burners, so that their temperature may be regulated to give the different temperatures desired in the different chambers. 20 The leer is provided with longitudinal stationary bars 43 and with endwise and vertically movable bars 44, mounted on rollers 45 in a manner similar to that of a usual rod-leer. 25 The movable bars may be shoved into the drawing-chamber beneath the supporting-bars 26 and between the tongs, the supporting-bars being lowered upon the leer-bars, which are then moved to carry the set of 30 sheets into the first leer-chamber. The rollers 45 may be mounted upon rocking shafts 46, as shown in Fig. 4, which are raised and lowered by link connections 47 with upper rock-shafts 48.

35 In order to preheat the pieces of glass or other material forming the baits, I preferably provide in the outlet-flue 49, leading from the top of the drawing-chamber, two sets of wheels 50, upon which are arranged movable 40 bars 51, upon which the bars 26, carrying the clamps or tongs 27, may rest at their ends. A set of the baits is thus heated, and after the bars with the drawn sheets have been taken into the leer from the drawing-frame 45 the upper bars 51 are moved forward to carry the new set of baits into the upper part of the drawing-chamber. The drawing-frame is lifted up until the bars 26 enter the slots in the end bars. The bars 51 are then drawn back, and the new baits are ready to be lowered 50 into the glass-bath to draw a new set of sheets.

The operation is preferably as follows: The ladle and trough 7 being in the position 55 shown in Fig. 4, the pot is lowered into position shown in dotted lines, the trough 7 tilting down. The ladle is then tilted to discharge its contents of glass into the trough and the pot. The pot is then preferably 60 lifted in parallel lines, the shields being in horizontal lowered position to protect the glass until it is of the proper temper. When ready for drawing, the shields are swung back, the drawing-frame is lowered until the set of baits enters the bath, and the frame is then 65

gradually raised to draw the sheets upwardly within the chamber. From the pot-chamber the sheets move up into the drawing-chamber above, which is inclosed to prevent the sheet from breaking. After the desired 70 length of sheets is obtained the drawing-frame may be stopped, the end-supporting bars 52 for the water-pipes 34 are lowered, and these pipes are shoved together to bring them in contact with the lower end portions 75 of the sheets. The pot is then lowered in parallel lines, and the flame beneath the pipes melts off the sheets and severs them from the glass of the bath. During the drawing operation the outer sheets serve to protect and 80 equalize the heat of the inner sheets, and thus prevent their warping, and for this reason the drawing of a plurality of sheets at the same time forms an important part of my invention. After the sheets are drawn and 85 severed I preferably tilt the pot, after a re-heating, if necessary, to discharge the glass into the small receptacle 21, and thus get rid of the faulty portion of glass remaining on the surface of the glass remaining in the pot. The 90 drawing-tools with the sheets depending therefrom are then lifted from the drawing-frame and the batch of sheets taken to the first leer-chamber. The drawing-frame is then moved up to take another set of baits 95 and when the pot is again charged is lowered and the operation repeated.

The advantages of my invention result from the simultaneous drawing of a plurality of sheets, from the manner of feeding the 100 glass into the pot and discharging the impurities from the pot after drawing, from the simple and effective arrangement for changing baits and feeding the sheets into the leer, the arrangement of the chilling devices, &c. 105

Many changes may be made in the form and arrangement of the parts without departing from my invention.

I claim—

1. The method of forming glass sheets consisting in simultaneously drawing a plurality of the sheets from a common bath of molten glass upwardly within an inclosed atmosphere common to all the sheets; substantially as described.

2. The method of drawing sheets, consisting in feeding glass into a separate pot or receptacle within a chamber, and simultaneously drawing a series of sheets upwardly within the inclosed atmosphere of the chamber; substantially as described.

3. The method of drawing glass sheets consisting in simultaneously drawing a series of sheets upwardly within a common drawing-chamber, and then passing said sheets through a gradually-decreasing temperature; substantially as described.

4. The method of forming glass sheets consisting in lowering a series of baits into a glass-bath, simultaneously raising the baits and

drawing the series of sheets, simultaneously chilling each sheet at or near the point of drawing and drawing the sheets upwardly within an inclosed atmosphere common to all said sheets; substantially as described.

5. The method of forming glass sheets, which consists in simultaneously drawing from a pot a series of sheets into an inclosed atmosphere common to all the sheets, then discharging from the pot the impure portions of the remaining glass, recharging the pot, and then drawing another series of sheets; substantially as described.

6. The method of forming glass sheets, which consists in simultaneously drawing a series of sheets into an inclosed atmosphere common to all the sheets, suspending the sheets in adjacent parallel planes, and then carrying them flatwise through a leer; substantially as described.

7. The method of drawing glass sheets consisting in lowering a series of baits into a common molten bath and simultaneously drawing the baits upwardly within an inclosed atmosphere common to all the sheets, whereby the outer sheets protect the inner sheets from warping; substantially as described.

8. The method of forming glass sheets consisting in simultaneously drawing a series of sheets upwardly within an inclosed atmosphere common to all the sheets, whereby the outer sheets protect the inner sheets from warping; substantially as described.

In testimony whereof I have hereunto set my hand.

J. H. LUBBERS.

Witnesses:

L. A. CONNER, Jr.,  
H. M. CORWIN.